

1

2,944,011

## SWEETENING HYDROCARBONS WITH DRIED CHROMIUM OXIDE

Peter B. Murray, Swarthmore, Pa., assignor to Sun Oil Company, Philadelphia, Pa., a corporation of New Jersey

No Drawing. Filed Dec. 10, 1956, Ser. No. 627,142

6 Claims. (Cl. 208—189)

This invention relates to the conversion of mercaptans contained in hydrocarbon materials, and more particularly to a manner of refining petroleum fractions containing mercaptans.

It is frequently desirable to treat hydrocarbon materials such as petroleum fractions in order to convert mercaptans contained therein into a less objectionable form. Thus for example, straight run or cracked gasoline may be treated in order to eliminate the bad odor caused by mercaptans normally contained in such fractions. Also, petroleum fuel oil compositions, for example cracked gas oils, may be treated in order to convert mercaptans which, if not converted, react with copper during use of the fuel oil, the resulting copper mercaptides having undesirable gel-forming properties.

In the conversion of mercaptans, for example to disulfides, by contact with a refining agent, it is desirable that the refining agent be capable of treating a large amount of hydrocarbon material. The present invention is advantageous in providing a refining agent which is capable of providing highly satisfactory conversion of mercaptans, while retaining its activity for such conversion during treatment of large amounts of hydrocarbon materials. The invention is further advantageous in that the refining agent is susceptible to regeneration without excessive difficulty to restore its high activity for conversion of mercaptans.

The treating agent employed according to the invention comprises chromium oxide which has been pretreated in a special manner which is required for satisfactory results. The treating agent can consist essentially of solid chromium oxide or it can comprise chromium oxide associated with other materials. Preferably, the treating agent comprises chromium oxide associated with a solid porous granular support or carrier. The treating agent is subjected to a drying operation prior to contacting with hydrocarbons containing mercaptans. The drying operation is essential, since it has been found that the life of the treating agent is disadvantageously short when the treating operation is not directly preceded by a drying operation.

The drying operation can be conducted in any suitable manner. It may for example involve heating with or without the aid of reduced pressure, to vaporize water. A dry gas capable of taking up water vapor can if desired be contacted with the treating agent to remove water therefrom. The drying operation is preferably performed by subjecting the treating agent to temperatures above the boiling point of water at the pressure involved, though this feature is not essential if a drying gas is used for example. At atmospheric pressure, the temperature is preferably at least about 250° F. At subatmospheric pressures, lower temperatures, e.g. down to 200° F. or lower can be employed. The duration of the drying is preferably sufficient to remove a major proportion of the water normally contained in the treating agent in equilibrium with the atmosphere. The duration is preferably at least one half hour, though shorter times are sufficient

2

under severer drying conditions. Usually, not more 10 hours will be required though longer times can be employed if desired.

It is further preferred according to the invention that the treating agent be subjected to a further heating operation which is carried out in the presence of gaseous oxygen. Any suitable oxygen containing gas, e.g. air, can be employed. The temperature of such contacting with oxygen is preferably within the approximate range

10 from 250° F. to 1500° F., and more preferably at least 750° F. The drying step and the contacting with oxygen can be conducted in a single operation, or if desired in separate operations comprising a drying step at relatively low temperature followed by a heating step at

15 higher temperature with introduction of gaseous oxygen into the heating zone. The time of heating in the presence of oxygen is preferably within the approximate range from one hour to ten hours, though other periods can be employed if desired.

20 Preferably the treating agent according to the invention is in a low state of hydration as a result of the pretreatment, since the absence of water contributes beneficially to the life and activity of the treating agent for conversion of mercaptans. It is also preferred that the

25 chromium in the treating agent should comprise large proportions of hexavalent chromium, present for example as chromium trioxide, since such chromium is generally more active for the purpose of the invention than chromium in lower valence states. Preheating in the presence

30 of oxygen to temperatures of at least about 750° F. for example is preferred in that it favors the formation of hexavalent chromium.

It has been found that the treating agent according to the invention has very high activity and long life in the 35 conversion of mercaptans. Thus for example 2000 bbls. of straight run gasoline or more can typically be rendered sweet to the doctor test per ton of treating agent containing 5% chromium trioxide. Treating agents containing greater proportions of chromium trioxide have

40 even longer life.

The hydrocarbon charged to the treated operation preferably contains little if any water, since water tends to decrease the life of the treating agent. Preferably therefore the hydrocarbon charge is dried prior to the treating 45 operation, in those cases where the charge ordinarily contains excessive amounts of water. Any suitable known method for dehydration of hydrocarbons can be employed prior to the treating step. Thus for example calcium chloride or other suitable known drying agent can be employed.

The hydrocarbon charge should be as free as possible of strong acids such as mineral acids. Thus generally the content of mineral acidity should be less than 100 p.p.m., and preferably is as close to zero as possible.

55 Accordingly, the charge should not be treated with a mineral acid prior to the treating operation according to the invention. Excessive amounts of mineral acid in the charge result in rapid deactivation of the treating agent, and also render the treating agent more difficult to regenerate.

The process according to the invention is carried out at a temperature below about 140° F. Excessively high temperatures should be avoided in order to avoid decomposition and darkening of the hydrocarbon charge 65 and also of the treating agent. The process is carried out in liquid phase, and elevated pressure is employed if necessary, though operation at atmospheric pressure is preferred. Preferably, the process is carried out by percolating the hydrocarbon charge through a stationary 70 bed of the treating agent, though other contacting methods as well known in the art can be employed if desired.

The process according to the invention is believed to involve oxidation of mercaptans to form disulfides. The oxygen necessary for this oxidation is supplied by the oxygen associated with chromium in the treating agent. Other oxidation reactions which occur in the presence of excessive amounts of gaseous oxygen are generally undesired, and are minimized when the oxygen associated with chromium is the principal or sole source of oxygen for the process. The hydrocarbon charge is preferably substantially free of gaseous oxygen. However, most hydrocarbon charge stocks as produced in ordinary petroleum refining do not contain excessive amounts of oxygen, and affirmative removal of oxygen is generally not necessary.

Any suitable support for the chromium oxide can be employed. Examples of suitable supports are silica gel, alumina, silica-alumina compositions, bauxite, clay, activated carbon, asbestos, kieselguhr, magnesium oxide, pumice, etc. In the case of bauxite, either ordinary bauxite or high- or low-iron bauxites as obtained in magnetic separation of bauxite can be employed. Any suitable manner of associating chromium oxide with the support can be employed, e.g. coprecipitation, impregnation, etc. Thus for example the support and the chromium compound can be coprecipitated from an aqueous solution, or the support, which may have been previously precipitated from an aqueous solution, can be impregnated with an aqueous solution of a chromium compound, etc. Examples of chromium compounds, aqueous solutions of which can be employed in precipitation or impregnation processes, are chromium oxides, e.g., chromium trioxide (chromic acid), and various compounds convertible thereto by heating, e.g., chromium acetate, chromium chloride, chromium sulfate, ammonium chromate, ammonium dichromate.

The treating agent according to the invention can be regenerated, after use in conversion of mercaptans, by contacting with steam or other inert vaporous or gaseous material to remove adsorbed hydrocarbons, and subsequently drying the treating agent or heating with oxygen in the manner previously described with regard to original preparation of the treating agent.

Little or no hydrogen sulfide is formed in the process according to the invention, the process involving oxidation of mercaptans to disulfides rather than decomposition of organic sulfur compounds to form hydrogen sulfides.

The amount of chromium oxide contained on the support can vary widely. In general, greater amounts of chromium oxide provide more satisfactory operation, longer life, etc. In the case of coprecipitated treating agents, as much as 70 weight percent of chromium oxide can if desired be incorporated in the treating agent. In the case of treating agents formed by impregnation, it is generally not feasible to incorporate more than 40 weight percent of chromium trioxide. Generally, it will be desired to incorporate at least one weight percent of chromium trioxide.

The support material, such as a silica-alumina composition, can be separately activated if desired by heating to a temperature for example within the approximate range from 1100° F. to 1300° F. for 2 to 16 hours in the presence of steam and air, the amount of steam in the activating gas being within the approximate range from 3 to 10 volume percent.

If desired, other metals can be associated with the chromium in the treating agent, for example strontium, iron, etc. However, chromium oxide provides highly satisfactory results in the absence of other metals.

The following example illustrates the invention:

*Example I*

A treating agent was prepared containing coprecipitated silica and alumina impregnated with 5 weight percent of chromium oxide. The weight proportion of silica to

alumina was 9 to 1. The silica-alumina composite was prepared according to standard procedure for preparation of synthetic silica-alumina cracking catalysts, as well known in the art, and the composite, which was about 10 to 20 mesh (United States sieve series), conformed to standard cracking catalysts.

The impregnation was performed by adding an aqueous solution of chromium trioxide to the silica-alumina composite in proportions equivalent to 56 milliliters of solution per 100 grams of composite, the weight ratio of chromium trioxide on the anhydrous basis to the composite being 4.9:100. A portion of the impregnated material was pretreated by heating to 900-1000° F. for one hour, while blowing air across the material. Directly following this pretreatment, 60 cc. of the impregnated composite were employed in a stationary bed as a treating agent for straight run gasoline containing essentially no mineral acidity and containing 0.006 weight percent of mercaptan sulfur.

The gasoline was passed through the bed at room temperature and atmospheric pressure and a liquid hourly space velocity of 15 volumes per volume of catalyst bed per hour. Three liters of doctor sweet product were obtained in 3½ hours. The treatment was then terminated. However, there was no sign of deactivation of the treating agent at the time of termination, indicating that considerably larger amounts of doctor sweet product could be obtained.

For comparison, another portion of the impregnated material, after an initial drying at 250° F. for 2 hours, was allowed to stand exposed to the atmosphere at room temperature for several days, thereby becoming hydrated by adsorption of water from the atmosphere. The treating agent was then used to treat another portion of the same straight run gasoline under the same conditions as in the case of the other portion of the impregnated material. The following results were obtained:

| 40                                         | Treating Agent Pretreatment | Liters of Doctor Sweet Product |
|--------------------------------------------|-----------------------------|--------------------------------|
| Heated with oxygen, 900-1,000° F., 2 hours | -----                       | >3                             |
| Exposed to atmosphere at room temperature  | -----                       | 1                              |

45 This table shows that it is essential to obtain good life, to dry the treating agent directly prior to the contacting with hydrocarbons.

Drying at lower temperatures in the absence of added oxygen is satisfactory in some instances. Thus, for example, drying at 250° F. for 2 hours is effective, if directly followed by hydrocarbon contacting, to provide longer life than in the case of an undried treating agent.

50 Results generally similar to those obtained in this example are obtained with other treating agents within the scope of the invention, e.g. bauxite impregnated with aqueous chromium nitrate and heated with added air to 1400° F. for 5 hours to obtain a composition containing 25 weight percent of chromium oxide, silica gel impregnated with aqueous ammonium chromate and 55 heated in the absence of added air to 400° F. for 15 hours, care being taken to avoid too rapid heating and spontaneous thermal decomposition, to obtain a composition containing 10 weight percent of chromium oxide, etc.

60 65 The low mineral acidity of the gasoline treated is an essential feature. In treating, under conditions described in Example I, a gasoline containing 0.006 weight percent (about 60 p.p.m.) of mercaptan sulfur and 150 p.p.m., for example, of sulfuric acid, the amount of doctor sweet 70 gasoline obtainable is much less than that obtained in Example I, and the regeneration of the treating agent is also more difficult.

75 Preferably, the amount of hexavalent chromium in the treating agent is about 35 to 100 weight percent based

on total chromium, and more preferably at least about 50 weight percent. Thus, for example, under the conditions of Example I, superior sweetening effect and life are obtained with 50 percent hexavalent chromium than with 25 percent.

The hydrocarbon charge stock which is refined according to the invention generally contains only a small amount of mercaptans. Typically, the amount is within the approximate range from 0.0005 to 0.05 weight percent, though other amounts are present in some instances.

The invention claimed is:

1. Process for sweetening hydrocarbons which comprises contacting hydrocarbons containing mercaptans and containing less than about 100 p.p.m. of mineral acidity in liquid phase at a temperature less than about 140° F. with a solid refining agent consisting essentially of material selected from the group consisting of dried chromium oxide and dried chromium oxide associated with a solid granular support, said refining agent containing 35 to 100% hexavalent chromium based on total chromium, thereby to selectively convert mercaptans to disulfides.

2. Process according to claim 1 wherein said refining agent is previously dried at a temperature of at least about 200° F. and above the boiling point of water at the pressure employed.

3. Process according to claim 1 wherein said refining

agent is previously contacted with gaseous oxygen at a temperature within the approximate range from 750° F. to 1500° F.

4. Process according to claim 1 wherein the chromium oxide is supported on a solid porous carrier.

5. Process according to claim 1 wherein said hydrocarbons are a gasoline fraction.

6. Process according to claim 1 wherein said hydrocarbons are a petroleum fuel oil fraction.

References Cited in the file of this patent

UNITED STATES PATENTS

|           |             |                |
|-----------|-------------|----------------|
| 10,055    | Brown       | Sept. 27, 1853 |
| 81,071    | De Gerbeth  | Aug. 18, 1868  |
| 190,762   | Jenny       | May 15, 1877   |
| 648,048   | Frasch      | May 8, 1900    |
| 713,475   | Mims        | Nov. 11, 1902  |
| 1,110,925 | Greenstreet | Sept. 15, 1914 |
| 1,318,061 | Ellis       | Oct. 7, 1919   |
| 1,590,965 | Downs       | June 29, 1926  |
| 2,325,115 | Egloff      | July 27, 1943  |
| 2,346,734 | Dempsey     | Apr. 18, 1944  |
| 2,351,094 | Blaker      | June 13, 1944  |
| 2,357,691 | Ruthruff    | Sept. 5, 1944  |

FOREIGN PATENTS

|         |               |              |
|---------|---------------|--------------|
| 143,193 | Great Britain | Feb. 3, 1921 |
|---------|---------------|--------------|